

## UNITED STATES PATENT OFFICE.

PIERRE JULIEN CLÉMENT MARGOTTON, OF NIORT, FRANCE.

## TANNING OF HIDES AND SKINS.

No Drawing.

Application filed July 26, 1921. Serial No. 487,622.

*To all whom it may concern:*

Be it known that PIERRE JULIEN CLÉMENT MARGOTTON, a citizen of the Republic of France, and resident of Niort, France (post office address Niort, Deux Sevres), have invented new and useful Improvements in the Tanning of Hides and Skins, which improvements are fully set forth in the following specification.

10 The present invention relates to the tanning of hides and skins, and more especially to hides intended to be used in the manufacture of gloves, by a series of operations which enable the tanning to be 15 effected in an extremely short time; the hides having first been subjected to working in a stream and tawed, and having been fleshed and pressed in the white.

To effect the tanning of dehaired hides, 20 they are passed, as subsequently explained, into a bath consisting of chromic acid, sulfuric acid and water. The object of the sulfuric acid is to activate the solution of chromic acid and to facilitate the penetration 25 of the bath into the interior of the hides. The proportion of chromic acid may be varied according to the weight of the hides; that of sulfuric acid, according to the weight of chromic acid introduced into 30 the bath. As regards the quantity of water, this is constant whatever the weight or the grain of the hides to be treated. For example, the following proportions may be adopted:

35 For 50 grams of dehaired hides,  
    Chromic acid\_\_ 2 grams.  
    Sulfuric acid\_\_ 2 cubic centimeters.  
    Water\_\_\_\_\_ 8 liters.

(This quantity of water will be used whatever 40 may be the weight and size of the dehaired hides.)

*Example 1.*

Bath for a small dehaired hide of 500 45 grams.  
    20 grams chromic acid.  
    20 cc. sulfuric acid. (These quantities may vary.)  
    3 liters water. (Constant quantity.)

*Example 2.*

Bath for a large dehaired hide.  
    40 grams chromic acid.  
    40 cc. sulfuric acid. (These quantities may 50 vary.)  
    3 liters water. (Constant quantity.)

The bath is contained in a suitable fulling tank or vessel, into which the dehaired hides are also introduced; and this tank, which is constructed to be rendered water-tight when closed, is then rotated by any desired means, its rotary movement causing the hides to slide one upon another and to strike heavily against the walls of the tank. In consequence, the bath liquid is alternately absorbed by and expelled from the hides, thus effecting an energetic fulling action which is assisted by the impact of the hides against the tank walls.

The hides remain in the fulling tank until 70 completely penetrated by the liquid, which condition can be ascertained by making incisions in the hides which should be yellow all the way through. They are thereupon removed from the tank and allowed to drip, and are then nailed on frames which are placed in a reaction chamber wherein the chromic acid in the hides is transformed into sulfate of chromium sesquioxide, in order to effect the tanning. In this chamber 75 they are enveloped in an atmosphere of sulfurous acid gas which, since it is heavier than air, is kept in motion by means of a fan; and they are allowed to remain therein until the reduction is complete, that is to say until they have turned blue all the way through, which can be ascertained by means of incisions. When the treatment is concluded, air is blown into the chamber to drive out the sulfurous acid gas, and the hides are 80 next treated to neutralize the sulfurous acid combined in their interior, so as to prevent them from becoming corroded.

For this purpose, a heated current of air 85 is caused to pass through a tank partly filled with ammonia in solution, the air taking up the ammonia vapors and then flowing into the reaction chamber where it envelopes the hides. The treatment is continued until the hides are neutralized or even slightly basic, 90 whereupon the chamber is again blown out and the hides withdrawn therefrom and washed in order to remove the ammonia. After washing, they are passed through a wringing machine to remove the excess 95 water, and are then again nailed upon frames and replaced in the reaction chamber; by which time they have been rendered unsusceptible to putrefaction, because of the above treatments.

The hides are next subjected to a second 100 tanning action in order to render them very

supple; this supplemental tanning action or 5 partial chamoising being effected with oil and being very light only. It can be carried out very easily in consequence of the small content of sulfate of chromium sesquioxide in the hides. In order to effect the immediate penetration of the oil into the interior of the hides, ordinary denatured alcohol is used; the hides being placed in the reaction 10 chamber and subjected to a current of hot air which has been caused to pass through a tank half full of alcohol. The alcohol vapors, in passing through the chamber, are absorbed by the water in the interior of the hides and 15 thus impregnate the latter; and to prevent the vapors from condensing in the interior of the chamber, the temperature thereof is kept at 30° C. Condensation may, however, be effected after the vapors have left the 20 chamber, and the alcohol thus recovered may be used again.

When the hides have been thoroughly impregnated with the alcohol, the operation is stopped, the chamber is blown out with air, 25 and the hides are removed from their frames and transferred to a suitable tilting vat containing oil in which they are submerged and which they readily absorb. After having been completely saturated by the oil, the 30 hides are dumped out of the tank upon a draining board, then wrung to remove the excess oil, and then re-nailed to their frames and put back in the reaction chamber. The latter is then heated to a temperature of 45° 35 to 50° C., and maintained at that temperature for an hour, during which time the alcohol is vaporized by the heat and carries off the water with it, leaving only the oil in the interior of the hides; this oil being oxidized 40 in the presence of the chromium sesquioxide and effecting a fresh tanning action which constitutes a partial chamoising.

The hides are now left for an hour in the reaction chamber and then removed from the 45 frames and transferred to an oil press, whereafter they are degreased, then scraped again, wrung and finally nailed to a drying floor.

It is thus possible to effect the tanning of 50 hides in a very short space of time; and the leather thereby obtained is much finer than chamois, the grain is closer and the hide less shaggy, the tanning being also more thorough since the hides are tanned twice, first with chromic acid and then with oil.

55 What I claim and desire to secure by Letters Patent is:—

1. A process of tanning, comprising the steps of subjecting the dehaired skins to the action of a tanning bath containing chromic

acid; treating the skins with sulfurous acid 60 gas in a closed receptacle to transform the chromic acid into sulfate of chromium sesquioxide; subjecting them to the action of ammoniacal vapors to force out the sulfurous acid gas; washing the skin with water until 65 the ammonia is removed, and then expelling the excess water; then subjecting them to the action of alcohol vapors; submerging the skins in oil; evaporating the alcohol from the skins and leaving the oil therein to be 70 oxidized in the presence of the chromium sesquioxide and to effect a fresh tanning action; and finally drying the skins.

2. In a process of tanning, the steps of 75 subjecting the dehaired skins to the action of a tanning bath containing chromic acid; then treating the skins with a substance which will convert the chromic acid into chromium sesquioxide; and then treating the skins with oil, thereby to oxidize the oil in 80 the presence of the chromium sesquioxide and to effect a fresh tanning action.

3. In a process of tanning, the steps of 85 subjecting the dehaired skins to the action of a tanning bath containing chromic acid; then treating the damp skins first with sulfurous acid and then with ammonia; removing the ammonia; and subjecting the skins to a fresh tanning action with oil.

4. In a process of tanning, the steps of 90 subjecting the dehaired skins to the action of a tanning bath containing chromic acid; then treating the damp skins first with sulfurous acid gas and then with ammoniacal vapors entrained in air; removing the ammonia; and subjecting the skins to a fresh 95 tanning action with oil.

5. In a process of tanning, the steps of 100 subjecting the dehaired skins to the action of a tanning bath containing chromic acid; then treating the damp skins first with sulfurous acid and then with ammonia; removing the ammonia; subjecting the skins to the 105 action of alcohol vapors; and then submerging them in oil and evaporating the alcohol, leaving the oil in the skins to be oxidized in the presence of the chromium sesquioxide formed consequent upon the action of the sulfurous acid on the chromic acid, whereby a fresh tanning action is effected.

In testimony whereof I have signed this specification in the presence of two subscribing witnesses.

PIERRE JULIEN CLÉMENT MARGOTTON. [L. S.]

Witnesses:

F. KRIBOULLEAU,  
MARCELLE BOULLERNE.